



US005079100A

# United States Patent [19]

Descamp et al.

[11] Patent Number: 5,079,100

[45] Date of Patent: Jan. 7, 1992

[54] WEAR RESISTANT COATINGS FOR  
ENGINE COMPONENTS AND A PROCESS  
FOR PRODUCING SUCH COATINGS

[75] Inventors: Martine Descamp, Villejuif; Yves C. L. A. Honnorat, Orsay; Michel M. Ruimi, Paris, all of France

[73] Assignee: Societe Nationale d'Etude et de Construction de Motors d'Aviation, Paris, France

[21] Appl. No.: 434,019

[22] Filed: Nov. 9, 1989

[30] Foreign Application Priority Data

Nov. 9, 1988 [FR] France ..... 88 14607

[51] Int. Cl.<sup>5</sup> ..... B32B 15/02

[52] U.S. Cl. ..... 428/552; 428/564;

428/627; 428/632; 428/678; 428/680; 428/934

[58] Field of Search ..... 428/627, 632, 639, 640, 428/678, 680, 934, 552, 554, 555, 556, 564

[56] References Cited

U.S. PATENT DOCUMENTS

- |           |         |                  |       |         |
|-----------|---------|------------------|-------|---------|
| 4,124,737 | 11/1978 | Wolfla et al.    | ..... | 428/640 |
| 4,275,124 | 6/1981  | McComas et al.   | ..... | 428/678 |
| 4,401,724 | 8/1983  | Moskowitz et al. | ..... | 428/678 |
| 4,741,975 | 5/1988  | Nair et al.      | ..... | 428/627 |
| 4,855,188 | 8/1989  | Garg et al.      | ..... | 428/627 |
| 4,873,152 | 10/1989 | Garg et al.      | ..... | 428/627 |
| 4,943,487 | 7/1990  | Benn et al.      | ..... | 428/678 |

## OTHER PUBLICATIONS

Chemical Abstracts, vol. 89, No. 16, Oct. 1978, p. 538, resume No. 137652w, Columbus, Ohio, US.

Primary Examiner—R. Dean

Assistant Examiner—George Wyszomierski

Attorney, Agent, or Firm—Oblon, Spivak, McClelland, Maier & Neustadt

[57]

## ABSTRACT

Engine components of steel or superalloy subject to wear from alternating friction at medium temperatures in the region of 700° C. are provided with a protective wear-resistant coating by

- electrophoretic deposition of a metal-ceramic structure comprising a mixture of from 85% to 50% of metallic powder and from 15% to 50% of ceramic powder, the metallic powder being a cobalt-based superalloy of type KC 25 NW or of M Cr Al Y wherein M represents at least one metal chosen from the group consisting of Ni, Co and Fe with the possible addition of Ta, and the ceramic powder being an oxide such as Al<sub>2</sub>O<sub>3</sub> or Cr<sub>2</sub>O<sub>3</sub>, a carbide such as SiC or Cr<sub>3</sub>C<sub>2</sub>, a nitride such as BN or TiN, or a boride such as TiB<sub>2</sub>;
- electrolytic pre-nickeling said deposit in an electrolysis bath at a pH between 6 and 8, and
- electrolytic nickelating said pre-nickled deposit in an acid bath of sulphamate type.

A further step of stress-relieving the nickelated deposit may be carried out at a temperature below 700° C.

6 Claims, 13 Drawing Sheets



G x 100

FIG. 1



G x 500

FIG. 2



G x 500

FIG. 3



G x 100

FIG. 4



G x 500-

FIG. 5



G x 500

FIG. 6



G x 100

FIG. 7



G x 200

FIG. 8



G x 500

FIG. 9



G x 100

FIG. 10



G x 500

 $e = 60$  to  $70 \mu\text{m}$ 

MCrALY

FIG. 11



G x 1000

FIG. 12



G x 100

FIG. 13



G x 500

 $e \approx 70 \mu\text{m}$   
HS 31

FIG. 14

Al<sub>2</sub>O<sub>3</sub>

Ni

 $e \approx 80 \mu\text{m}$ 

G x 500

FIG. 15



FIG. 16



FIG. 17



FIG. 18



FIG. 19



G x 25

FIG. 20a



G x 200

FIG. 20b



G x 1000

FIG. 20c



G x 25

FIG. 21a



G x 200

FIG. 21b



G x 1000

FIG. 21c



G x 25

FIG. 22a



G x 200

FIG. 22b



G x 1000

FIG. 22c



G x 25

FIG. 23a



G x 200

FIG. 23b



G x 1000

FIG. 23c



FIG. 24



FIG. 25a



FIG. 25b



FIG. 25c



FIG. 26



FIG. 27

**WEAR RESISTANT COATINGS FOR ENGINE  
COMPONENTS AND A PROCESS FOR  
PRODUCING SUCH COATINGS**

**BACKGROUND OF THE INVENTION**

**1. Field of the Invention**

The present invention relates to engine components of steel or superalloy comprising a coating for preventing wear when subjected to alternating friction at medium temperature, i.e. in the vicinity of 700° C., and also to a process for obtaining such coatings.

In turboshaft engines, for example, particularly those intended for aircraft, several parts subjected to temperatures from 400° C. to 800° C. undergo alternating frictions against which they must be protected. Some examples of where such frictions occur are as follows:

the centering of the combustion chamber inlet diffuser on the preceding compressor stage;

the support of an upstream inner platform of the high pressure turbine guide on the downstream flange of the combustion chamber;

the positioning of the outer platform of the high pressure turbine guide on the front and rear flanges of the high pressure turbine casing;

the fixing flange of turbine sectors on the high pressure turbine casing;

the centering of the exhaust cone on the turbine outlet casing.

**2. Summary of the Prior Art**

An attempt has been made to form a coating at these various places which would compensate for wear and provide a hard wear-resistant layer. For this purpose, the components at these places were subjected to a localized electrolytic deposition of cobalt with a chromium oxide Cr<sub>2</sub>O<sub>3</sub> phase in the cobalt bath. It has been observed, however, that although this type of coating is effective in the first two examples mentioned above, it is not at all so in the last three cases where wear and flaking, and even breaking away, of the coating has occurred.

It has been possible to correlate these observations with the temperatures experienced at the different areas, and it has been determined that electrolytic depositions of cobalt with a dispersed phase of chromium oxide only behave satisfactorily below a temperature of 700° C. on a continuous basis, beyond which, flaking occurs.

**SUMMARY OF THE INVENTION**

The aim of the invention is to solve the problem of providing a wear-resistant coating which remains effective beyond 700° C. on a continuous basis.

To achieve this, the invention proposes to effect a metallic deposition of M Cr Al Y type, wherein M is selected from the group comprising Ni, Co, Fe and mixtures thereof with the possible addition of Ta, dispersed with ceramic particles chosen from the group comprising oxides, carbides, nitrides and borides. This type of coating may be obtained by electrophoretic deposition but it is necessary, in order to make it adherent to the substrate, to increase the proportion of nickel in the deposit. The invention therefore further proposes to consolidate the deposition by adding nickel electrolytically, and then to perform a heat treatment at a relatively low temperature, so as to stress-relieve the coating.

The most commonly used electrolytic nickel-plating processes are generally carried out in acid baths containing nickel sulphamate. However, it has been observed, when performing electrolytic nickel-plating

5 onto a composite electrophoretic deposition of M Cr Al Y metal and ceramic in a sulphamate bath, that the electrophoretic layer was systematically destroyed. The cause of this seems to originate from the acidity of the bath (pH below 4) which produces a chemical reaction 10 of the acid solution with the powder deposit.

On the other hand, if it is desired to use a nickel-plating bath having a pH close to 7, another problem has to be faced, which is the poor cathodic yield due essentially to the instability of the bath resulting from the 15 precipitation, at PH=5.5, of nickel salts in the form of hydroxide Ni (OH)<sub>2</sub>.

Another difficulty with such metal-ceramic deposits consolidated by nickel-plating comes from the fact that, to obtain an adequately resistant layer, one is tempted to

20 carry out the electrophoretic powder deposition to a considerable thickness. However, whatever the nature may be of the nickel bath used, very thick depositions (above 40 microns) have a tendency to react badly to nickel plating. On the other hand, it has been observed that 25 it is easier to nickel electrophoretic deposits of small thickness, the intensity and the voltage remaining constant throughout the operation.

In effect, electrolytic nickel-plating is performed at a constant current density, but the mechanical brittleness 30 of thick layers of the initial electrophoretic deposit and their electrical resistance result in the occurrence of breakdown phenomena (mechanical and electrical), and therefore short-circuits, if one chooses to operate with too high a current density.

35 The invention, which resides in providing an electrophoretic metal-ceramic deposition consolidated by electrolytic nickel plating, is thus made possible by the judicious selection of the parameters of the successive operations of electrophoresis and electrolytic nickel plating, and also 40 by carrying out, between the electrophoresis and electrolytic nickel plating in an acid medium, an electrolytic prenickeling in a medium close to neutrality, so as to create in the electrophoretic deposit a nickel film which commences consolidation of the deposit without damaging it, and also acts as a bonding base for the nickel subsequently deposited.

According to the invention, therefore, there is provided 45 an engine component of steel or superalloy having a protective coating for providing wear-resistance against alternating friction at medium temperatures, said protective coating comprising a metal-ceramic structure formed from a cobalt based superalloy of KC25NW type or a mixture of metallic powders of M Cr Al Y type wherein M represents at least one metal selected from the group consisting of Ni, Co, and Fe, with the possible addition of Ta, and from ceramic powders selected from the group consisting of oxides (preferably Al<sub>2</sub>O<sub>3</sub> and Cr<sub>2</sub>O<sub>3</sub>), carbides (preferably SiC and Cr<sub>3</sub>C<sub>2</sub>), nitrides (preferably BN and TiN), and borides (preferably TiB<sub>2</sub>), said metal-ceramic structure being formed by electrophoretic deposition and being consolidated and bound to the component by electrolytic nickel plating and stress-relieving heat treatment at a temperature below 700° C.

Further according to the invention there is provided 55 a process for forming a protective coating on an engine component of steel or superalloy, particularly a nickel-based alloy, for providing wear resistance against alter-

nating friction in the dry state at medium temperatures the process comprising the steps of:

- a) forming a deposit on said component by electrophoresis, said deposit having a metal-ceramic structure comprising a mixture of from 85% to 50% by mass of metallic powder and from 15% to 50% by mass of ceramic powder, in which said metallic powder is a cobalt-based superalloy of KC25NW type or is of M Cr Al Y wherein M represents at least one metal selected from the group consisting of Ni, Co, and Fe with the possible addition of Ta, and said ceramic powder is selected from the group consisting of carbides, oxides, nitrides and borides;
- b) subjecting said deposit to electrolytic prenickeling in an electrolysis bath at a pH of from 6 to 8; and
- c) after said prenickeling, subjecting said deposit to electrolytic nickel in an acid bath of sulphamate type.

Preferably the duration of the electrophoresis step a) is between 5 and 60 seconds and said deposit has a thickness of from 10 to 40 microns depending on the grain size of the powders used.

Preferably, the electrolytic prenickeling step b) is carried out in an electrolysis bath containing ammonium lactate and having its pH kept between 6 and 8 by the addition of soda.

In order to produce a protective coating having a substantial thickness, for example 100 microns, a series of relatively small thickness deposits are formed one on top of another by repeating the sequence of steps (a),(b) and (c), either with a stress-relieving treatment after each nickel step or with only one stress-relieving heat treatment after the last nickel step, until the desired thickness has been reached. In contrast, with the knowledge previously available to the specialist the tendency would have been towards carrying out the electrophoretic deposition to produce the required thickness in a single operation, followed by the operations of pre-nickeling, nickel and stress-relieving, which would have resulted in the nickel problems mentioned earlier.

The process in accordance with the invention may also include a pre-nickeling step and a nickel step before subjecting the component to the electrophoresis step to form the metal-ceramic deposit.

#### BRIEF DESCRIPTION OF THE DRAWINGS

FIGS. 1 to 3 are photomicrographs at magnifications of X100, X500, and X500 respectively of a section through a first example (sample 325) of a metal-ceramic coating produced in accordance with the invention wherein the coating comprises a mixture of Co Ni Cr Al Y Ta + 20% Al<sub>2</sub>O<sub>3</sub> of grain size less than 25 microns the photomicrographs being taken after micrographic attack in a bath containing HF 15%, HNO<sub>3</sub> 15%, and H<sub>2</sub>O 70%.

FIGS. 4 to 6 are photomicrographs at magnifications of X100, X500, and X500 similar to those of FIGS. 1 to 3 but showing a second example (Sample 331) of a coating produced in accordance with the invention, the coating comprising Co Ni Cr Al Y Ta of grain size less than 25 microns + 20% Cr<sub>3</sub>C<sub>2</sub> of grain size less than 45 microns.

FIGS. 7 to 9 are similar photomicrographs at magnifications of X100, X200, and X500 showing a third example (Sample 281) of a coating produced in accordance with the invention.

FIGS. 10 to 12 are photomicrographs at magnifications of X100, X500 and X1000 showing a fourth example (Sample 285) of a coating produced in accordance with the invention, the coating comprising Co Ni Cr Al Y Ta of grain size below 25 microns + 20% TiB<sub>2</sub> of grain size less than 4 microns.

FIGS. 13 to 15 are photomicrographs at magnifications of X100, X500, and X500 showing a fifth example (Sample 469) of a coating produced in accordance with the invention in which the coating comprises KC25NW and 20% Al<sub>2</sub>O<sub>3</sub>, the metal and ceramic powders being of grain size smaller than 25 microns.

FIGS. 16 and 17 are photomicrographs at magnifications of X200 and X500 showing a sixth example of a coating produced in accordance with the invention and comprising Co Ni Cr Al Y Ta + 20% Al<sub>2</sub>O<sub>3</sub> of grain size less than 25 microns, with a sub-layer of electrolytic nickel.

FIGS. 18 and 19 are photomicrographs at magnifications of X200 and X500 showing a seventh example (Sample 328) of a coating produced in accordance with the invention, the coating comprising Co Ni Cr Al Y Ta + 30% Al<sub>2</sub>O<sub>3</sub> with a sub-layer of electrolytic nickel.

FIGS. 20 to 23 are photomicrographs showing the results of grid tests on various samples, the photographs (a) being at X25 magnification, the photographs (b) being at X200 magnification, and the photographs (c) being at X1000 magnification. The photographs 20a, 20b, 20c are of sample 326 (example 1, single deposit coating). The photographs 21a, 21b, 21c are of sample 333 (Example 2, single deposit coating). The photographs 22a, 22b, 22c are of sample 325 (Example 1, double deposit coating). The photographs 23a, 23b, 23c are of sample 331 (Example 2, double deposit coating).

FIG. 24 is a diagram showing the principles of the apparatus used for carrying out dry alternating friction tests on test samples.

FIGS. 25a, 25b and 25c are views showing the shape of the test samples used in the apparatus of FIG. 24.

FIG. 26 is a theoretical graph showing the volume worn in terms of time using the friction test apparatus.

FIG. 27 is a comparative diagram comparing the performance of coatings produced in accordance with the invention with that of three other coatings of known type in terms of the volume worn on running-in.

#### DESCRIPTION OF THE PREFERRED EMBODIMENTS

Numerous tests under different operational conditions were carried out following a common general procedure. Test pieces consisting of 1 dm<sup>2</sup> plates of alloy Z12 C13 —AFNOR standard (trade name: AISI 410) having the following composition by weight: 0.12% C, 13% Cr, and Fe the remainder were used as substrates for protective coatings produced in accordance with the invention.

After preparation in a known manner involving cleaning and polishing, the test pieces were mounted in the cathodic position in an apparatus of known type permitting electrophoretic deposition. In all the cases tested, the electrophoresis bath used comprised a base of isopropanol/nitromethane, with a soluble metallic or organometallic salt as electrolyte.

The metal-ceramic mixture to be deposited consisted, in all of the examples, of 80% by weight of metallic powder (either of cobalt based superalloy or of M-Cr Al Y type, as defined earlier) and 20% by weight of ceramic powder.

In the case of the example using cobalt-based superalloy (sample No. 469), KC25NW (AFNOR standard) was used, this being obtained under the trade name HS 31 and having a composition, by weight, of Cr 24 to 26%; Ni 10 to 12%; W 7 to 9%; and Co the remainder.

In the case of the examples using M-Cr Al Y powder (samples Nos. 281,285,286,325,328,331), the powder used was that obtained under the name AMDRY 67 having a composition, by weight, of Cr 23 to 25%; Ni 8.5 to 11%; Al 6 to 8%; Ta 4 to 6%; Y 0.4 to 0.8%; and Co the remainder.

After mixing in the proportions mentioned above, in one example the metal-ceramic mixture had the composition, by weight:

Co 35.69%; ceramic 20%; Cr 19.37%; Ni 8.65%; Al 8.06%; Ta 7.84%; Y 0.39%.

Various concentrations of metal-ceramic mix between 40 g/l and 100 g/l were tested, and good results were obtained for a 60 g/l concentration.

The electrophoretic deposition was carried out with an electric potential  $U=500$  V, and for a period between 5 and 60 seconds with magnetic stirring.

After the electrophoretic deposition, the test pieces were placed in an electrolysis tank where they were subjected to pre-nickeling in a near neutral bath comprising:

$\text{NiSO}_4$  70 g/l

$\text{H}_3\text{BO}_3$  15 g/l

$\text{NH}_4\text{Cl}$  15 g/l

Ammonium lactate 10 g/l (8.5 ml/l).

The pre-nickeling was conducted under the following conditions:

pH maintained between 6.8 and 7 by the addition of

$\text{NaOH}$ ;

current density between 0.2 and 0.5 A/dm<sup>2</sup>;

temperature between 20° C. and 30° C.;

anodes of pure silver;

duration from 10 to 30 minutes.

The test pieces were then subjected to nickel plating in an acidic bath (pH close to 4) composed of 75 g/l of Ni metal in the form of Ni sulphamate, 18 g/l nickel chloride  $\text{NiCl}_2$ , 6H<sub>2</sub>O, 35 g/l  $\text{H}_3\text{BO}_3$ , and a wetting agent, the nickel plating being carried out under the following conditions:

current density between 0.5 and 1 A/dm<sup>2</sup>;

duration from 10 to 60 min;

temperature between 20° C. and 50° C.

The test pieces were then subjected to a nickel stress-relieving treatment at 600° C. under vacuum for 4 hours.

Within this general procedure, the following parameters were subjected to variations:

the nature of the ceramic powder;  $\text{SiC}$ ,  $\text{Cr}_3\text{C}_2$ ,  $\text{Al}_2\text{O}_3$ ,  $\text{BN}$ ,  $\text{TiN}$ ;

the grain size of the powders: a first series of tests were conducted with powders of diameter ranging from 40 to 50 microns, and a second series of tests were conducted with powders of a diameter less than 25 microns.

the temperature during the pre-nickeling and nickel plating steps;

the current density and duration for each of the pre-nickeling and nickel plating operations.

Table 2 (at the end of the description) summarizes the various operational conditions tested during the pre-nickeling and nickel plating operations. In each case, two or three layers (each comprising one electrophoretic depo-

sition, pre-nickeling in a near neutral bath and nickel plating in an acidic bath) were deposited in forming the coating.

## FIRST EXAMPLE

### Samples 325 and 326

An electrophoretic deposition of a powder mixture of  $\text{Co Ni Cr Al Y Ta}$  and 20% by weight of alumina  $\text{Al}_2\text{O}_3$ , the metallic and ceramic powders each having a grain size below 25 microns, was formed on a substrate of Z 12 C 13 in the manner described above.

Pre-nickeling in a near neutral bath containing ammonium lactate was then carried out at 30° C. for 20 mins at a current density of 0.1 A/dm<sup>2</sup>, and in order to obtain a substantial nickel percentage per layer this was followed by nickel plating in a sulphamate bath for a period of 60 mins.

The nickel plating was divided into two stages having different parameters (temperature and current density). In the first stage (C1) the temperature was 30° C. and current density 0.5 A/dm<sup>2</sup>, and in the second stage (C2) the temperature of the bath was raised to 50° C. and the current density to 1 A/dm<sup>2</sup>.

For sample 325, two consecutive layers each comprising a metal-ceramic electrophoretic deposition, a pre-nickeling and a nickel plating as described above were deposited, followed by a nickel stress-relieving treatment at 600° C. under vacuum for 4 hours.

Under the conditions described above it was found, after analysis, (see Table 2) that the final composition of the coating was an alloy comprising about 50% of metal-ceramic powder and 50% electrolytic nickel.

FIG. 1 shows that the coating is even and that its thickness ranges from 35 to 50 microns. The photograph of FIG. 2, at greater magnification, was taken in an area of 35 micron average thickness and shows a good distribution of the particles of alumina in the electrolytic nickel. The photograph of FIG. 3, at the same magnification as FIG. 2, was taken in an area of 50 micron thickness and also evidences the satisfactory distribution of the metallic and ceramic particles in the thickness of the coating.

Sample 326 has only a single layer coating and was used for comparative grid behaviour tests.

## SECOND EXAMPLE

### Samples 331 and 333

The metallic powder used was identical to that of the first example, and the grain size was also the same. The ceramic powder was a chromium carbide  $\text{Cr}_3\text{C}_2$  of grain size between 20 and 45 microns (20% by weight of the metallic and ceramic powder mixture). The operational conditions observed in forming the coating were the same as in the preceding example.

It was found that with two layers (sample 331), one obtains (FIG. 4) a homogeneous coating of a thickness between 40 and 70 microns. The photographs of FIGS. 5 and 6 show that the metal-ceramic alloy/substrate interface is chemically sound, just as in the foregoing example (FIGS. 2 and 3), but exhibits a few pores. There are also a number of pores within the alloy coating itself which are not filled in during the nickel plating. The distribution of the particles of M-Cr Al Y and chromium carbide in the metal-ceramic alloy is even and homogeneous.

Sample 333 was formed with a single layer coating for use in comparative grid behaviour tests.

## THIRD EXAMPLE

## Sample 281

The same Co Ni Cr Al Y Ta metallic powder was used as in the previous examples, with the incorporation into it of 20% by weight of boron nitride BN, the grain size of the latter being between 30 and 60 microns.

Three layers were deposited in succession under the following operational conditions for each layer:

electrophoretic deposition of the metal-ceramic mix as described earlier;

pre-nickeling at 30° C. for 30 mins and 0.1 A/dm<sup>2</sup>;

two-stage nickelizing comprising a first stage for 30 mins at 50° C. and 0.5 A/dm<sup>2</sup>, and a second stage for 45 mins at 50° C. and 1A/dm<sup>2</sup>.

After stress-relieving the coating at 600° C. for 4 hours under vacuum, the coating alloy formed consisted of 49% Co Ni Cr Al Y Ta and BN mixture and 51% electrolytic nickel. The wear-resistant coating (FIG. 7) was of homogeneous thickness ranging between 60 and 70 microns.

The grains of BN, larger than those of the M-Cr Al Y metal, were nevertheless evenly distributed in the coating, and the nickel was diffused homogeneously towards the substrate.

## FOURTH EXAMPLE

## Sample 285

The same Co Ni Cr Al Y Ta metallic powder was used as in the previous examples, with the admixture of 20% by weight of titanium diboride TiB<sub>2</sub>, the grain size of the latter being below 4 microns. Three layers were deposited under operational conditions identical to those used in the third example.

The alloy coating formed comprised a little more than 50% M Cr Al Y Ta and TiB<sub>2</sub> and a little less than 50% electrolytic nickel. The thickness of the wear-resistant coating (FIG. 10) is uniform over the entire surface of the sample, close to 54 microns. The titanium diboride particles of very small grain size are particularly well distributed, as are the grains of M-Cr Al Y Ta in the electrolytic nickel medium.

## FIFTH EXAMPLE

## Sample 469

The cobalt based superalloy KC25NW (trade name HS31) with a grain size below 25 microns was used as the metallic powder, and was mixed with 20% by weight of alumina Al<sub>2</sub>O<sub>3</sub> of grain size less than 25 microns.

Three successive layers were deposited and stress-relieved to form a coating using the same operational conditions for electrophoretic deposition, pre-nickeling, nickelizing and stress-relief as were used in examples 3 and 4.

FIGS. 13 to 15 show the evenness of the thickness of the coating between 70 and 80 microns, and the homogeneous distribution of the particles of HS 31 and alumina in the electrolytic nickel.

## SIXTH EXAMPLE

## Sample 286

In this example the same M-Cr Al Y metallic powder as used in examples 1 to 4 was mixed with 20% by weight of alumina of grain size below 25 microns.

In this case it was desired to obtain a final coating with a thickness greater than that of the previous exam-

ples. To achieve this, rather than depositing more than three layers of the metal-ceramic material, it was decided to form, between the substrate and the metal-ceramic layers, a sub-layer of electrolytic nickel. This sub-layer was obtained after acid pickling of the substrate by deposition of a flash of nickel in a Wood nickelizing bath comprising:

NiCl<sub>2</sub>, 6H<sub>2</sub>O: 240 g/l

Nickel metal: 59 g/l

HCl: from 80 to 110 ml/l at d:1.16.

Pre-nickeling was carried out at ambient temperature for 6 mins at a current density between 4 and 4.5 A/dm<sup>2</sup>. The deposition of the nickel flash was followed by an electrolytic deposition of nickel in a sulphamate bath under the same conditions described earlier for the sulphamate nickelizing step (c) of the coating process in accordance with the invention.

After this electrolytic nickelizing, the metal-ceramic coating process of the invention was performed in conditions identical to those used in examples 3 to 5, i.e. with the deposition of three layers, and the final layer being followed by stress-relief under vacuum for 4 hours at 600° C. The photographs of FIGS. 16 and 17 show the appearance of the coating obtained. The sub-layer of electrolytic nickel has a thickness close to 25 microns, whereas the thickness of the metal-ceramic layers is between 80 and 90 microns. The particles of M-Cr Al Y and the alumina are evenly distributed, and the inter-diffusion of the electrolytic nickel and of the wear-resistant coating has created a particularly efficient keying of the metal-ceramic layers.

## SEVENTH EXAMPLE

## Sample 328

As in the previous example a sub-layer of electrolytic nickel was formed under the same conditions, increasing the duration of the nickelizing so as to obtain a sub-layer about 45 microns thick.

Following this operation a metal-ceramic deposition comprising 70% by weight of the M-Cr Al Y powder and 30% alumina of grain size below 4 microns was carried out, two layers being deposited in the same conditions as in the previous example. The resulting wear-resistant coating had a thickness of from 50 to 60 microns which, together with the thickness of the nickel sub-layer, provided a total coating thickness of between 95 and 105 microns.

It will be seen from Table 2 and FIG. 19 that the metal-ceramic coating still contains about 50% nickel, although it is distributed in a slightly less homogeneous manner than in the previous examples.

## TEST RESULTS

The adherence and wear behaviour of the coatings formed in accordance with the invention were tested, and the results of some of these tests are indicated below.

## Bending and Grid Tests

These were carried out on 15×100 mm test pieces to characterize the adherence of the coatings obtained in samples 325,326,331,333.

The results of the bending tests are summarized in Table 1.

TABLE 1

| TEST<br>SPECIFICATIONS                          | OBSERVA-<br>TIONS 326-<br>333- SINGLE<br>LAYER DEPOSIT                            | RESULTS                            |                            |
|-------------------------------------------------|-----------------------------------------------------------------------------------|------------------------------------|----------------------------|
|                                                 |                                                                                   | DOUBLE LAYER<br>DEPOSIT            | RESULTS                    |
| Folding on cylindrical tube of diameter 12.7 mm | Grain size: diameter 10 to 25 microns<br>Theoretical thickness 100 to 150 $\mu$ m | No cracks.<br>Satisfactory results | No cracks.<br>Good results |
| Folding on cylindrical tube of diameter 8 mm    | Thickness of coating ~ 50 microns<br>Elongation 11%                               | No cracks.<br>Satisfactory         | No cracks.<br>Good results |

Similar tests were carried out on batches 285,469,286 15 and 328. The results were of equally good quality, even for batches 286 and 328 having a nickel sub-layer of substantial thickness.

Grid tests were carried out on single layer deposits (samples 326 and 333) and double layer deposits (sample 20 325 and 331) on samples scored with crossed lines.

On the single layer coatings (sample 326—FIGS. 20a, 20b, 20c; sample 333—FIGS. 21a, 21b, 21c), no breaking away of the protective coating was observed, even though the base metal of the substrate was reached.

On the double layer coatings (sample 325—FIGS. 22a, 22b, 22c; sample 331—FIGS. 23a, 23b, 23c), the results were even better, as only the first layer of the coating was affected by the cross-lining.

These cross-lining tests illustrate the good attachment to the substrate of the coatings produced in accordance with the invention.

#### Dry Alternating Friction Tests

These were carried out on homogeneous pairs of raw coated test pieces and were conducted in comparison with other known types of wear resistant coating.

The equipment used is shown in FIG. 24, and the form of the test pieces is shown in FIGS. 25a, 25b and 25c.

The test pieces consist of members 1 having a diametrical boss 2 of convex shape on which the wear resistant coating is formed. For the friction tests coatings were used similar to those formed in examples 1 and 2 and corresponding respectively to samples 325 (Ni Co Cr Al Y Ta+20%  $\text{Al}_2\text{O}_3$  and 331 (Ni Co Cr Al Y Ta+20%  $\text{Cr}_3\text{C}_2$ ).

Two identical test pieces 1 are attached to a pair of arms 3a and 3b so that the coated bosses 2 are in face to face contact with each other. The two arms 3a and 3b are pivoted on axles 4, the arm 3a being caused to execute an alternating angular movement through an angle  $\alpha$  by means of an eccentric 5, while the arm 3b is biased against the arm 3a by means of a spring blade 6 exerting a load which may vary from 1.7 to 70 daN. The ends of 50 the arms 3a and 3b holding the test pieces 1 are arranged inside a heated enclosure 7 enabling the friction tests to be conducted over a temperature range of from 20° C. to 600° C. The friction frequency may be set between 0 and 50 Hz and the amplitude of movement may range from 0.1 to 2 mm.

In FIG. 26 the curve (1) shows the stabilized wear rate “ $V_u$ ”, whereas the extrapolation (to  $t=0$ ) of the straight line representing the stabilized wear rate indicates the volume  $V_a$  worn during the period of wear-in.

The curve (2) established at  $V_u=0$  is intended to identify the critical wear pressure  $P_{cu}$  which is the ratio

of the applied load to the worn surface of the test piece in the event of jammed wear ( $V_u=0$ ).

Table 3 below is a comparison of the values  $U_a$ ,  $V_u$  and  $P_{cu}$  at 20° C., 250° C., 400° C. and 600° C. for homogeneous pairs of test pieces having the following wear resistant coatings:

Test No. 1: Wear-resistant coatings of the invention 25 as in example 1 (sample 325).

Test No. 2: Wear-resistant coatings of the invention as in example 2 (sample 331).

Test No. 3: Wear-resistant coatings of Amdry 996 (trade name) having the composition, by weight:

30 Al: 6 to 8%  
Cr: 23 to 25%  
Ni: 8.5 to 11%  
Ta: 4 to 6%  
Y: 0.4 to 0.8%

35 Co: the remainder  
mixed with 20% by weight of alumina and consolidated at high temperature (1150° C.) for 4 hours as known in the art.

Test No. 4: Wear-resistant coatings formed by plasma 40 deposition of HS31 (trade name) (AFNOR standard KC 25 NW) as known in the art.

Test No. 5: Wear-resistant coatings of Tribomet 104C (trade name) formed by electrolytic deposition of cobalt-chromium carbide as known in the art.

FIG. 27, which is derived from Table 3, shows a comparison of the volumes worn on wearing-in as a function of temperature for the five tests mentioned above. Curves 1 to 5 plot the values of above-mentioned tests 1 to 5.

It will be noted from Table 3 and FIG. 27 that, at ambient temperature, the rate of wear of the coatings formed in accordance with the invention is slightly higher than that of some of the known coatings. However, this behaviour clearly improves as the temperature rises.

Indeed, between 250° C. and 600° C. the coating of the invention containing 20% alumina (sample 325—curve No. 1) exhibits, as a consequence of its low wear on wearing-in and of the relatively high critical pressure, very good wear resistance which is better than, or at least equivalent to, the other coatings tested.

The coating formed in accordance with the invention comprising chromium carbide (sample 331—curve No. 2) exhibits characteristics of much the same quality above 400° C., in which range its wear resistance becomes greater than that of Amdry 996+ $\text{Al}_2\text{O}_3$  (curve No. 3) and of Tribomet 104C (curve 5), and close to that of HS 31 plasma (curve No. 4).

FIG. 27 therefore illustrates the considerable benefit of consolidation by low temperature electrolytic nickel-ing, the resulting coatings being greatly superior to those of curve 3 formed using the high temperature heat

ties regarding the nature, the form, and the concentration of the wear-resistant Particles, as well as the consolidation treatment (e.g., chromium-plating, cobalt-plating, alloying, etc.).

TABLE 2

| Mixture % by weight                            | Powder Grain size - diameter (Ø) microns | Sample No.       | OPERATION (1) PL/NS | θ (°C.) | Operating conditions cd (A/dm/time (min.)) | deposit reference | m electro phoresis in total per deposit | Total electrolytic Ni % per deposit | thickness (microns)  |
|------------------------------------------------|------------------------------------------|------------------|---------------------|---------|--------------------------------------------|-------------------|-----------------------------------------|-------------------------------------|----------------------|
| Co Ni Cr Al                                    | Ø ≤ 25                                   | 325 (2 deposits) | PL(b) NS(c1)        | 30°     | 0,1/20                                     | 1st               | 9,2/16,8                                | 45                                  | 35 to 50 homogeneous |
| Y Ta + Al <sub>2</sub> O <sub>3</sub> (20%)    |                                          | 326 (1 deposits) | C NS(c2)            | 50°     | 1/30                                       | 2nd               | 8,4/17                                  | 50,5                                |                      |
| Co Ni Cr Al                                    | Ø MCrALY ≤ 25                            | 331 (2 deposits) | PL(b) NS(c1)        | 30°     | 0,1/20                                     | 1st               | 12,5/21,7                               | 42                                  | 60 to 70 homogeneous |
| Y Ta + Cr <sub>3</sub> C <sub>2</sub> 20 (20%) | Ø CR <sub>3</sub> C <sub>2</sub> ≤ 25    | 233 (1 deposits) | C NS(c2)            | 50°     | 1/30                                       | 2nd               | 12,1/22,1                               | 45                                  |                      |
| Co Ni Cr Al                                    | Ø MCrCALY 25                             | 281              | PL(b)               | 30°     | 0,1/30                                     | 1st               | 12,2/21,6                               | 44                                  | 60 to 70             |
| Y Ta + 20% BN                                  | 30 ≤ Ø BN ≤ 60                           |                  | NS(c)               | 50°     | 0,5/30                                     | 2nd               | 10,2/20,8                               | 51                                  | microns              |
| Co Ni Cr Al                                    | Ø MrCALY ≤ 25                            | 285              | PL(b)               | 30°     | 0,1/30                                     | 1st               | 6,4/18,3                                | 65                                  | 60 to 70             |
| Y Ta + 20% TiB <sub>2</sub>                    | Ø TiB ≤ 4 microns                        |                  | NS(c)               | 50°     | 0,5/30                                     | 2nd               | 11,6/22,4                               | 48                                  | microns              |
| KC 25 NW (H 531)                               | Ø KC25 NW ≤ 25                           | 460              | PL(b)               | 30°     | 0,1/30                                     | 1st               | 8,1/21,2                                | 62                                  | 70 to 80             |
| 20% Al <sub>2</sub> O <sub>3</sub>             | Ø AL 0 25                                |                  |                     | 50°     | 0,5/30                                     | 2nd               | 10,4/25                                 | 58                                  | microns              |
| Co Ni Cr Al                                    | Ø ≤ 25                                   | 286              | PL(b)               | 30°     | 0,1/30                                     | 1st               | 7,3/17                                  | 57                                  | 80 to 90             |
| Y Ta + 20% Al <sub>2</sub> O <sub>3</sub>      |                                          |                  | NS(c)               | 50°     | 0,5/30                                     | 2nd               | 9/19,2                                  | 53                                  | microns              |
| Co Ni Cr Al                                    | Ø MCrAlY ≤ 25                            | 328              | PL(b)               | 30°     | 0,1/30                                     | 1st               | 8,7/17,2                                | 49                                  | 50 to 60             |
| Y Ta + 30% Al <sub>2</sub> O <sub>3</sub>      | Ø Al <sub>2</sub> O <sub>3</sub> ≤ 4     |                  | NS(c)               | 50°     | 0,5/30                                     | 2nd               | 8,6/18,2                                | 53                                  | microns              |
|                                                |                                          |                  |                     |         | 1/45                                       | 3rd               | 8,7/26,3                                | 67                                  |                      |

(1) Step (a): Electrophoresis operational conditions identical in all cases: U = 500 V; t = 5s

Step (b): PL = Prenickeling in a neutral ammonium lactate bath 6.8 pH 7

Step (c): NS = Nickel in a nickel sulphamate acid bath pH = 4.

TABLE 3

| Deposits Examined                                                                                             | Test Temperatures |      |     |         |      |     |         |    |      |         |    |      |
|---------------------------------------------------------------------------------------------------------------|-------------------|------|-----|---------|------|-----|---------|----|------|---------|----|------|
|                                                                                                               | 20° C.            |      |     | 250° C. |      |     | 400° C. |    |      | 600° C. |    |      |
|                                                                                                               | Va                | Vu   | PCU | Va      | Vu   | PCU | Va      | Vu | PCU  | Va      | Vu | PCU  |
| 1 Co Ni Cr Al<br>Y Ta + 20% Al <sub>2</sub> O <sub>3</sub><br>Ex 325                                          | 200               | 5450 |     | 26      | 13,1 | 15  |         | 18 |      | 10      |    | 36   |
| 2 Co Ni Cr Al<br>Y Ta + 20% Cr <sub>3</sub> C <sub>2</sub><br>Ex 331                                          | 200               | 4600 |     | 280     | 1030 |     | 33      |    | 11,5 | 21      |    | 15,6 |
| 3 Amdry 996<br>+ 20% Al <sub>2</sub> O <sub>3</sub><br>thermally<br>consolidated<br>at 1150° C.<br>for 1 hour | 1000              | 150  |     |         | 125  |     | 800     |    |      | 2,95    |    |      |
| 4 HS 31 plasma                                                                                                | 200               | 220  |     | 270     | 125  |     | 30      |    |      | 15      |    |      |
|                                                                                                               | 200               | 220  |     | 270     | 125  |     | 30      |    |      | 15      |    |      |
| 5 T 104 C                                                                                                     | 0                 | 250  |     | 330     |      | 4   | 170     |    | 5,7  | 7       |    | 23   |
|                                                                                                               | 0                 | 250  |     | 330     |      | 4   | 170     |    | 5,7  | 7       |    | 23   |

Ua: Volume worn during wearing-in ( $10^{-3}$  mm<sup>3</sup>)

Vu: Stabilized rate of wear ( $10^{-3}$  mm<sup>3</sup>/h)

PCU: Critical wear pressure (MPa)

treatment (1150°/4 hours).

Equivalent results (not described here) have been obtained for coatings containing nitrides or borides (samples 281 and 285), and also for samples 286 and 328 including a sub-layer of electrolytic nickel.

These good results in the hot state make this wear-resistant coating treatment of considerable interest for components of complex shape which must be consolidated at medium temperatures.

Any person skilled in the art will understand that 65 these examples are for guidance only. The marriage of two deposition techniques so different as electrophoresis and electroplating opens up a vast choice of possibili-

We claim:

1. An engine component of steel or superalloy having a protective coating for providing resistance against wear from alternating friction at temperatures in the range of about 400° to 800° C. line 6, said protective coating comprising a metal-ceramic structure formed from:
  - a cobalt based superalloy powder comprising 24-26 wt. % Cr, 10-12 wt. % Ni, 7-9 wt. % W and the remainder Co or a mixture of MCrAlY metallic powder wherein M represents at least one metal

selected from the group consisting of Ni, Co and Fe with the possible addition of Ta; and  
 b) ceramic powder selected from the group consisting of oxides, carbides, nitrides and borides, said metal-ceramic structure having been obtained by electrophoretic deposition and having been consolidated, said coating further comprising electrolytic nickel which binds said metal-ceramic structure to the component and which comprises 42-67 wt % of said coating, said coating having been subjected to a stress-relief heat treatment.

2. An engine component according to claim 1, wherein said ceramic powder is selected from the group consisting of oxides of aluminum and chromium, carbides of silicon and chromium, nitrides of boron and titanium, and titanium boride.

3. An engine component according to claim 1, wherein the amount of said ceramic powder in said metal-ceramic structure is from 15% to 50% by weight, and the grain size of said metallic and ceramic powders is below 60 microns.

4. An engine component according to claim 3, wherein the grain size of said powders is below 25 microns.

5. An engine component according to claim 1, wherein said metallic powder has the following composition, by weight:

Cr: 23 to 25%  
 Ni: 8.5 to 11%  
 Al: 6 to 8%  
 Ta: 4 to 6%  
 Y: 0.4 to 0.8%  
 Co: the remainder

10 and said metallic powder is mixed with from 15 to 50%, by weight, of said ceramic powder, said metal-ceramic structure being electrophoretically deposited on the component in a time of not more than 60 seconds using an electric field of from 100 to 500 V/cm and a bath 15 containing a mixture of Isopropanol and Nitromethane, less than 0.1 g/l of a soluble metallic or organometallic salt as electrolyte, and from 40 to 100 g/l of said mixture of metallic and ceramic powders, and said deposited metal-ceramic structure having been consolidated by a 20 galvanic deposition of electrolytic nickel followed by said stress-relieving treatment.

6. An engine component according to claim 1, wherein beneath the wear-resistant coating there is a layer of electrolytic nickel formed by Wood pre-nickeling carried out at a current density between 4 and 5 25 A/dm<sup>2</sup> for from 5 to 6 minutes, followed by nickel in a sulphamate bath at a current density between 3 and 5 A/dm<sup>2</sup> for from 20 to 40 minutes.

\* \* \* \* \*

30

35

40

45

50

55

60

65

UNITED STATES PATENT AND TRADEMARK OFFICE  
CERTIFICATE OF CORRECTION

PATENT NO. : 5,079,100

Page 1 of 2

DATED : JANUARY 7, 1992

INVENTOR(S) : MARTINE DESCAMP ET AL

It is certified that error appears in the above-identified patent and that said Letters Patent is hereby corrected as shown below:

Column 2, line 15, delete "PH=5.5", insert --pH=5.5--.

Column 3, line 14, delete "prenickeling", insert  
--pre-nickeling--;  
line 16, delete "prenickeling", insert  
--pre-nickeling--;  
line 23, delete "prenickeling", insert  
--pre-nickeling--.

Column 8, line 24, after "600°C.", start new paragraph.

Column 9, line 37, delete "wear resistant", insert  
--wear-resistant--;  
line 42, delete "wear resistant", insert  
--wear-resistant--.

Column 10, line 23, delete "wear resistant", insert  
--wear-resistant--;  
line 43, delete "electroIytic", insert  
--electrolytic--.

Column 11, Table 2, after "Step (b): PL =", delete  
"Prenickeling'", insert --Pre-nickeling--.

Column 12, line 2, delete "Particles", insert --particles--.

Column 14, Claim 5, line 21, delete "stress-relieving", insert  
--stress-relief heat--.

UNITED STATES PATENT AND TRADEMARK OFFICE  
**CERTIFICATE OF CORRECTION**

PATENT NO. : 5,079,100

Page 2 of 2

DATED : January 7, 1992

INVENTOR(S) : Martine Descamp, et al.

It is certified that error appears in the above-identified patent and that said Letters Patent is hereby corrected as shown below:

Column 14, claim 6, line 23, after "is", insert --present--.

Signed and Sealed this

Twenty-eighth Day of June, 1994

Attest:



BRUCE LEHMAN

Attesting Officer

Commissioner of Patents and Trademarks